# EUROPEAN PATENT APPLICATION

(11) **EP 0 231 418 A1**
(43) Date of publication of application: **12.08.1987**
(21) Application number: 86101503.0
(22) Date of filing: 05.02.1986
(51) Int. Cl.: G03C 1/78, G03C 1/80

(54) **Sulfonated lithium cation exchanged polystyrene photographic films**

(71) Applicant: THE DOW CHEMICAL COMPANY, Midland Michigan 48640-1967 (US)
(72) Inventor: Ryan, Kevin J., Granville Ohio 43023 (US)
(74) Representative: Sternagel, Hans-Günther, Dr.

(57) **Abstract**

Photographic films comprising a base film of oriented polystyrene at least one surface of which is highly sulfonated and lithium cation exchanged.

## Description

This invention relates to styrene polymer photographic films and a method for making them.

It is known from Canadian Patent No. 674,921 that photographic films can be prepared from a polystyrene film base if an acrylic copolymer anchoring layer and a gelatin subbing layer are added to the film base before a photographic gelatin emulsion is added. U.S. Patent No. 2,872,318, suggests that the above anchoring layer can be eliminated if a subbing layer is applied from a special mixture of solvents.

Photographic films prepared by these processes are expensive because of the multiplicity of steps involved in their manufacture.

The use of other film bases for photographic purposes has been suggested in U.S. Patent No. 2,805,173 wherein polyethylene terephthalate is used and U.S. Patent No. 3,112,199 wherein isotactic polypropylene is used. These patents show that anchoring layers and subbing layers can be eliminated if the polymer surface is treated with a solution of chlorosulfonic acid and then aminated with various amines before a photographic gelatin emulsion is applied. Photographic films prepared by the teachings of U.S. Patent No. 2,805,173 are expensive, however, due to the high cost of the polymer base. Photographic films prepared by the teachings of U.S. Patent No. 3,112,199 lack the required stiffness for normal film processing and handling.

When attempts are made to sulfonate polypropylene and polyethylene terephthalate films to a hgih degree of sulfonation which is necessary for good adhesion, it is found that the film surface turns dark brown or black in the case of polypropylene and crumples away to a powder in the case of polyethylene terephthalate.

In U.S. Patent No. 3,725,109 a method is claimed for producing a photographic film form biaxially oriented films of styrene polymers by sulfonating them with a sulfur containing compound to produce a film having a high degree of sulfonic acid groups on the surface of the film. It has now been discovered that the quality of photographic film produced according to the process of U.S. Patent No. 3,725,109 may vary depending on the composition of the photographic gelatin emulsion employed.

A process for sulfonating the surface of polystyrene and exchanging the hydrogen ions in the sulfonated groups with metal ions is disclosed in British Patent No. 1,100,712.

The present invention resides in an article comprising 1) an oriented styrene polymer film having at least one surface thereof sulfonated, and 2) a photosensitive gelatin layer adhered to said surface; and wherein at least some of the sulfonate groups of said surface are neutralized by lithium cation exchange to provide improved adhesion of the gelatin layer to the oriented styrene polymer film.

The present invention also resides in a method of making a photographic film comprising the steps of sulfonating at least one side of an oriented polystyrene film, and neutralizing at least some of the sulfonate groups on said film with lithium cations such that the amount of neutralized sulfonate groups present on the film surface is sufficient to provide improved adhesion of a photographic gelatin layer thereto.

The present invention is basically a method for improving the adhesion of photographic gelatin emulsion to film formed from styrene polymer resins by sulfonating the fiom and by contacting the film with a lithium ion source thereby exchanging lithium ions for the hydrogen ions of the sulfonate groups. More particularly, it now has been found that photographic films can be produced from biaxially oriented films of styrene polymer resins by sulfonation to provide sufficient sulfonic acid groups on the film surface and then contacting the film with a lithium ion source to thereby replace at least some of the hydrogen ions on the sulfonic acid groups with lithium cations. By this process, the adhesion of the photographic gelatin emulsion to the film is increased over the degree of adhesion obtained by the sulfonation treatment only. The subsequent application of a photographic gelatin emulsion layer to the film surface results in a photographic film that is economical to make, has good dimensional stability during photographic processing and has good adhesion between the film and the gelatin layer. Additionally, the present invented composition accumulates markedly reduced amounts of static electricity thereby minimizing contamination due to accumulation of dust particles.

The polymer films to which this invention is directed are those known to the art and comprise those oriented films formed from styrene polymer resins. Non-oriented sytrene polymer films lack the structural strength which is necessary in photographic film applications.

Suitable films include those composed of styrene polymer resins and blends thereof with other resins and components which are employed to prepare films having specific physical characteristics desired in photographic film applications.

The term "styrene polymer resin" refers to polystyrene, copolymers of styrene with one or more copolymerizable ethylenically unsaturated monomers, or blends or grafts of polystyrene with synthetic elastomeric polymers. The term "styrene" is used to denote not only styrene but also alkyl-substituted derivatives of styrene such as α-methylstyrene. Examples of suitable styrene polymer resins are polystyrene, high impact polystyrene, acrylonitrile styrene copolymers, acrylonitrile butadiene styrene copolymers, methyl methacrylate-styrene copolymers, poly-α-methylstyrene, or copolymers of styrene and α-methylstyrene

Mixtures of styrene polymer resins as well as mixtures of ethylene polymer resins can be used.

The term "ethylene polymer resin" refers to polyethylene or copolymers of ethylene with one or more copolymerizable ethylenically unsaturated monomer. Suitable ethylene polymer resins include high density polyethylene, medium density polyethylene, low density polyethylene, chlorinated polyethylene, ethylene-higher alkene copolymers, ethylene-vinyl acetate copolymers, ethylene-vinyl chloride copolymers, ethylene-ethyl acrylate copolymers, and ethylene-acrylic acid copolymers and ionomers.

A specific film which finds good utility as a photographic film comprises a blend of styrene polymer resin, an ethylene polymer resin and an inorganic filler. Films of the type are taught, for example, in British Patent No. 1,257,512 and U.S. Patent No. 3,993,718. Preferably, the inorganic filler is titanium dioxide, and the blend contains greater than about 50 percent by weight of styrene polymer resin. More preferably, the blend also contains an elastomer polymer compound such as polybutadiene, a styrene-butadiene rubber, or an acrylonitrile-butadiene rubber to improve the physical properties of the film.

A more preferred film comprises from 78 to 88 weight percent sytrene polymer resin, from 3 to 6 weight percent ethylene polymer resin, from 3 to 6 weight percent of an elastomer compound, and from 6 to 10 weight percent titanium dioxide. Most preferably, such blend is prepared from styrene homopolymer or thermoplastic styrene-butadiene copolymer (high impact polystyrene), ethylene homopolymer and an elastomeric styrene-butadiene star block copolymer compatibilizer and titanium dioxide. The individual blend components and the overall blend can also include other additives which are normally incorporated into resin blends such as stabilizers, anti-static agent, plasticizers, colorants, and anti-oxidants.

As is well known from the literature (e.g., "Encyclopedia of Polymer Science," vol. 2, pages 339 to 373) biaxial orientation increases the tensile strength of polymer films in general and for polystyrene film it raises the range of ultimate tensile strength from 24,100 to 82,700 kPa (3,500 to 12,000 lb/in²) in both the machine direction and the transverse direction. Therefore, the films used in this invention are oriented styrene polymer resin films having a tensile strength in the stated range with or without impact strength modifiers of the type set forth above.

These oriented styrene polymer films are sulfonated on at least one side to produce sulfonic acid groups directly attached to the polymer film. Preferably, a high concentration of sulfonic acid groups are directly attached to the polymer film. Next, the sulfonic acid groups may be neutralized with a lithium cation. When these films are coated with a photosensitive gelatin or emulsion layer on the lithium metal ion neutralized sulfonated side of the film, the result is a photographic film of good durability with good adhesion of the gelatin to the base film and additionally, demonstrating reduced static charge build-up.

If desired, the polymer film can be sulfonated and lithium ion neutralized on both sides. Subsequently, both sides of the film may be coated with gelatin or emulsion layers. For example, one surface may be coated with one or more photosensitive gelatin layers and the back side of the film may be coated with an anti-halation or other gelatin layer.

For the purposes of this invention, the term "high concentration of sulfonic acid groups" means a range from 0.4 to 13 micrograms of sulfur trioxide equivalents per square centimeter of film. A most preferred range is from 5 to 10 micrograms of sulfur trioxide equivalents per square centimeter.

The above film is sulfonated in any suitable manner. For example, the film is vapor phase sulfonated with sulfur trioxide gas in a pure or dilute form to produce a film having a high concentration of sulfonic acid groups directly attached to the styrene polymer. It is preferred to sulfonate the film by moving it through a blast or curtain of sulfur trioxide gas in the absence of water or water vapor. This technique provides a method with great speed, uniformity, and no complications such as removal of solvents, etc. Alternatively, the film is passed through an atmosphere (versus a blast or stream of gas) of gaseous sulfur trioxide. In this technique slower speeds may be necessary to give adequate contact time between the film and the gas.

The sulfur trioxide gas can be used pure but since sulfur trioxide boils at 44.8°C it is difficult to keep it in the vapor state. The preferred method is to dilute vapors of sulfur trioxide with a dry inert gas such as air, carbon dioxide, nitrogen, and the like. The SO₃, in the inert gas, can range from 1 to 15 percent by weight.

Another method of sulfonating the styrene polymer film is to treat it with a solution of SO₃ dissolved in an inert liquid solvent. Typical useful inert liquid solvents are hydrocarbon solvents such as hexane, heptane, petroleum ether, kerosene, and the like. One technique for accomplishing this is taught, for example, in British Patent No. 1,100,712.

The SO₃ in the above solvents can range from 1 to 25 percent by weight SO₃ but it is preferred to use a lower range of from 1 to 5 percent by weight SO₃.

In the foregoing sulfonation processes the temperature can range from -20°C to 60°C with the preferred temperature range being from 20°C to 40°C.

The pressure at which the sulfonation is carried out can be atmospheric, superatmospheric, or subatmospheric. Because of the convenience, it is preferred to carry out the sulfonation at atmospheric pressure or at slightly elevated pressures of from 1.03 to 1.73 kg/cm² (1 to 10 pounds per square inch gauge).

After the film is sulfonated to the desired degree it is brought into contact with a lithium cation source and at least some and preferably substantially all the hydrogen ions on the sulfonic acid groups are replaced with lithium cations.

In order to cause ion exchange to occur, the sulfonated film is merely dipped into or otherwise brought into contact with a source of lithium ions such as a lithium metal salt solution. Suitable salts include LiCl, LiNO₃, Li₂SO₄, as well as any other source of lithium ions. Sufficient lithium cations should be provided to replace the desired amount of hydrogen ions contained on sulfonic acid groups present on the film. British Patent No. 1,100,712 teaches a method for performing the ion exchange treatment. Enough lithium ions are exchanged to result in improved adhesion of the gelatin layers. Preferably, from 10 to 100 percent of the surface sulfonate groups are exchanged with lithium cations.

In some instances, sulfonated films may first be treated with ammonia to replace the hydrogen atoms on the sulfonic acid groups. The ammonium cations can be replaced with a lithium cation in the same manner as employed for the hydrogen ion resulting in an ultimate product wherein hydrogen ions are replaced by lithium cations.

As an alternative procedure for ion exchange, the lithium cations may be contained in a gelatin or emulsion, such as a photosensitive gelatin and ion exchange allowed to occur when the gelatin is applied to the sulfonated film.

After ion exchange treatment, the film may be coated with any one of a number of commercially available photographic gelatin emulsions and dried. These gelatins include the photosensitive gelatins and other photographic gelatin emulsions employed as adhesive materials and the like. The film in the form of a roll can be unwound and dipped into the gelatin one or more times in order to build up a photosensitive layer of suitable thickness. The complete film is then allowed to dry for a sufficient period of time to allow the gelatin layer to harden.

The prepared photographic films have anti-static properties and have good wet and dry adhesion between the photosensitive gelatin and the film base as indicated by a pressure sensitive tape test.

### Examples

In the following examples, a sulfonated polystyrene film is prepared which includes neutralization with ammonia. The ammonia neutralized sulfonated film is then treated with a 0.1 N aqueous solution of metal compounds, further identified in Table I to exchange the ammonium cation with the metal cation.

The relative adhesion of a photosensitive gelatin layer to the polystyrene film is measured by a wet adhesion test. In the test, the film is coated with a photosensitive gelatin composed of water, gelatin, methanol, formaldehyde and saponin. The film is passed through developing chemicals as in normal photographic processing. A grid is then scribed with four prong fork through the gelatin to expose the polystyrene substrate. A cork or rubber eraser is then pressed and rubbed across the grid. The degree of adhesion is rated by the relative amount of gelatin removed from the film. The ratings range from 1 through 5 with a rating of 1 indicating essentially no gelatin loss and a rating of 5 indicating a loss of from 25 to 100 percent of the emulsion is removed.

The base film employed in the test is a Trycite® brand, biaxially oriented, surface sulfonated, polystyrene film available from The Dow Chemical Company. Films to be ion exchanged are contacted with the aqueous solution for one hour, rinsed with deionized water, dried for about 16 hours at ambient temperature, and coated with the gelatin layer (8 mil). Results of the above-described test are contained in Table I.

Sample numbers C1 through C8 are comparative examples.

## Claims

1. An article comprising
1) an oriented styrene polymer film having at least one surface thereof sulfonated, and
2) a photosensitive gelatin layer adhered to said surface;
and wherein at least some of the sulfonate groups of said surface are neutralized by lithium cation exchange to provide improved adhesion of the gelatin layer to the oriented styrene polymer film.

2. The article of Claim 1 wherein the amount of sulfonate groups present on the film surface is sufficient to provide from 0.4 to 13 micrograms of sulfur trioxide per square centimeter of film.

3. A method of making a photographic film comprising the steps of sulfonating at least one side of an oriented polystyrene film, and neutralizing at least some of the sulfonate groups on said film with lithium cations such that the amount of neutralized sulfonate groups present on the film surface is sufficient to provide improved adhesion of a photographic gelatin layer thereto.

4. The method of Claim 3 wherein the amount of sulfonate groups present on the film surface is sufficient to provide from 0.4 to 13 micrograms of sulfur trioxide equivalents per square centimeter of film.

5. The method of Claim 3 wherein the sulfonate groups of said surface are first neutralized by contact with ammonium ions and the ammonium ions then exchanged with lithium cations.

6. The method of Claim 3 wherein the sulfonate groups are neutralized by exchange with a lithium cation prior to application of the photosensitive gelatin layer.

7. The method of Claim 3 wherein on two surfaces sulfonate groups have been neutralized by exchange with a lithium cation.
